

Patented Jan. 14, 1936

2,027,750

# UNITED STATES PATENT OFFICE

2,027,750

## COPPER BASE ALLOY

Elmer L. Munson, Naugatuck, Conn., assignor to  
The American Brass Company, Waterbury,  
Conn., a corporation of Connecticut

No Drawing. Application October 20, 1934,  
Serial No. 749,276

10 Claims. (Cl. 148—21.2)

This invention relates to a copper base alloy containing copper, nickel, aluminum and beryllium.

It is one object of the invention to provide 5 a copper base alloy that has a combination of hardness, strength, ductility and a wide heat treating temperature range not found in other copper base alloys.

The foregoing and other objects will appear 10 from the following description and appended claims.

Several copper base alloys now in commercial use may be hardened and strengthened by the heat treating process known as precipitation or 15 age hardening treatment. Of these alloys two most important are the copper-nickel-aluminum alloy and the copper-nickel-beryllium alloy of the following approximate compositions:

|           | Per cent | Per cent  |       |
|-----------|----------|-----------|-------|
| 20 Copper | 94.0     | Copper    | 97.25 |
| Nickel    | 5.0      | Nickel    | 0.50  |
| Aluminum  | 1.0      | Beryllium | 2.25  |

Alloys of the above and similar compositions have certain objectionable characteristics which 25 do not appear in the new alloy which I have discovered. For example, the copper-nickel-aluminum alloy cannot be satisfactorily hardened at temperatures below about 325° C., while my new alloy can be heat treated at temperatures as low as 250° C. and consequently at less 30 expense. Again the copper-nickel-beryllium alloys have a heat treating temperature range extending from about 250° C. to about 325° C. which is a rather narrow range for use by the 35 fabricating trade and is a source of trouble when the heat treating time and (or) temperature is not closely regulated. The hardness and several other mechanical property values of the 40 copper-nickel-beryllium alloys reach a peak somewhere in the neighborhood of 300° C., depending upon the amount of cold working and time of heating. If the applied heat is materially below 250° C. or materially above 325° C., the hardness and other characteristics are not 45 satisfactory for commercial usage. In other words in the heat treatment of the above described copper-nickel-aluminum alloys and copper-nickel-beryllium alloys the temperature must be closely regulated with respect to the selected 50 temperature, and similarly the time must be closely defined. My new alloy does not require such close regulation of the heat treatment because variations of fifty degrees within the heat 55 treating temperature range do not seriously influence the hardness and other mechanical properties. In other words, there is a gradual increase in the mechanical property values from about 250° C. to about 550° C. About 550° C., the mechanical property values drop off until a 60 temperature of about 800° C. is reached, where

the metal, after quenching, is sufficiently soft to readily permit of cold working.

Many of the copper rich quaternary alloys of 5 copper, nickel, aluminum and beryllium have no properties which make them any better than the more simple binary or ternary alloys, but I have discovered a narrow range of composition in which these alloys possess the desirable characteristics of the previously known alloys of these metals and which, in addition, are free 10 from several undesirable features.

The most valuable composition range is approximately

|           |                |    |
|-----------|----------------|----|
| Copper    | 91.75 to 96.75 | 15 |
| Nickel    | 2.0 to 5.0     |    |
| Aluminum  | 0.5 to 2.0     |    |
| Beryllium | 0.75 to 1.25   |    |

When the percentages of nickel, aluminum and (or) beryllium materially exceed the maximum limits of these narrow ranges the alloy 20 cannot be fabricated into sheets, wire, rods, and tubes by the usual cold working methods such as rolling and drawing.

If the nickel, aluminum and (or) beryllium 25 contents are materially lower than the minimum limit, the resulting alloy can be cold worked commercially into wrought forms but will not develop the advantageous hardness, strength and ductility characteristic of the alloys within the 30 specified limits.

However, when only the beryllium content is lowered, my new alloy still shows better mechanical properties than the previously mentioned commercial copper-nickel-aluminum 35 alloy. A composition such as approximately

|           |                |    |
|-----------|----------------|----|
| Copper    | 90.25 to 97.25 |    |
| Nickel    | 2.0 to 7.0     |    |
| Aluminum  | 0.5 to 2.0     |    |
| Beryllium | 0.25 to 0.75   | 40 |

is of value for certain purposes.

A preferred specific alloy for tensile strength, hardness and ductility is one comprising approximately 94.5% copper, 3.5% nickel, 1.0% 45 aluminum, and 1.0% beryllium.

A useful alloy which can be produced at more moderate cost is one comprising approximately 95% copper, 3.5% nickel, 1.0% aluminum and 0.5% beryllium. 50

In the manufacture of my new copper base alloy the aluminum and beryllium may be added to the nickel and copper in the form of an addition alloy, such for example as one containing beryllium and aluminum in the proper proportions or as alloys of beryllium and/or aluminum with copper. The alloy is cast in chill or other molds and the ingots or shells may be hot and (or) cold rolled or drawn to the desired size and shape. The cast ingots or shells 60

can also be extruded or forged, if desired. If, at any stage, it is desired to soften the alloys for working purposes, this may be accomplished by heating preferably to about 800° C. (although a certain degree of softening will occur at any other temperature between approximately 550° C. and the melting point), and then rapidly cooling, preferably by an immediate quench in water. Hardening of finished articles made from the new alloy can be accomplished by heating within the temperature range approximately 250° C. to 550° C. for a period of from 1/2 hour to 2 hours. This treatment of the new alloy will raise the Rockwell hardness value to about "G" 100 and the tensile strength to about 130,000 pounds per sq. in. with an elongation of about 2% in 2 inches.

If so desired, the new alloy can be hardened automatically while in commercial service if the operating temperature is within the wide temperature range aforementioned.

My experiments have indicated that the nickel content should exceed the sum total of the aluminum plus beryllium content to secure the maximum hardness and strength.

An important advantage of an alloy made in accordance with the present invention is that the amount of beryllium required is only about one-half the quantity necessary in the prior copper-nickel-beryllium alloy to obtain nearly as great hardness and tensile strength values. At the present time, beryllium metal is more or less rare and expensive. Therefore, this reduction in beryllium content means that the base metal cost of the new alloy will be about 60 percent less than that of the prior alloy at current metal prices. This reduction is reflected in a lower sales price for the new alloy and consequently permits more extensive use of same in fields heretofore considered prohibitive due to the high cost of the prior copper-nickel-beryllium alloy.

Another advantage of an alloy made in accordance with the present invention is the greater softness of the annealed material in comparison with that of the copper-nickel-beryllium alloy. For example, the Rockwell hardness of my new wrought alloy after annealing at 800° C. for 1/2 hour followed by a quench in water is about "G" 12, while the Rockwell hardness of the copper-nickel-beryllium alloy similarly annealed and quenched is about "G" 25. This increased softness of my new copper-nickel-aluminum-beryllium alloy will permit greater reductions between anneals and with somewhat less die wear when drawn into wire or tubes than is possible with the copper-nickel-beryllium alloys.

Another advantage embodied in my invention is that afforded during the casting operation by the presence of the protective aluminum film on the surface of the molten metal which helps to prevent the loss of valuable beryllium by volatilization. In the copper-nickel-beryllium alloy some loss of the expensive element beryllium occurs by volatilization when the metal is molten prior to and during the pouring operation.

All of these characteristics combined with the excellent corrosion resistance of the copper base alloys containing nickel and aluminum make my

new alloy particularly suitable for such articles as non-sparking tools, hardware, knives, chisels, springs, wire screens, tubes, gears, terminals, clips, bolts, nuts, coins, clock parts, jewelry, chains, valves, hinges and many other articles. 5

Having thus set forth the nature of my invention, what I claim is:

1. An alloy composed of copper, nickel, aluminum and beryllium in proportions substantially within the following ranges: 10

|           | Percent         |
|-----------|-----------------|
| Copper    | 91.75 to 96.75  |
| Nickel    | 2.0 to 5.0      |
| Aluminum  | 0.5 to 2.0      |
| Beryllium | 0.75 to 1.25 15 |

2. An alloy comprising approximately 94.5% copper, 3.5% nickel, 1.0% aluminum and 1.0% beryllium.

3. A copper base alloy comprising approximately 95% copper, 3.5% nickel, 1.0% aluminum and 0.5% beryllium. 20

4. A copper base alloy composed of copper, nickel, aluminum and beryllium in proportions substantially within the following ranges: 25

|           | Percent         |
|-----------|-----------------|
| Copper    | 90.25 to 97.25  |
| Nickel    | 2.0 to 7.0      |
| Aluminum  | 0.5 to 2.0      |
| Beryllium | 0.25 to 0.75 30 |

5. A copper base alloy which is capable of extensive drawing, rolling and other forms of hot and cold working composed of 2.0% to 7.0% nickel; 0.5 to 2.0% aluminum; 0.25 to 1.25% beryllium, and the balance substantially copper. 35

6. A copper base alloy which has been hardened by heat treatment composed of 2.0% to 7.0% nickel; 0.5 to 2.0% aluminum; 0.25 to 1.25% beryllium, and the balance substantially 40 copper, in which the nickel content exceeds the aluminum and beryllium content.

7. A copper base alloy characterized by being hardenable by heat treatment composed of 2.0% to 7% nickel; 0.5 to 2.0% aluminum; 0.25 to 1.25% beryllium, and the balance copper, in 45 which the nickel content is approximately in the ratio of 3 1/2 to 1 aluminum and approximately the same amount of beryllium as aluminum.

8. A copper base alloy composed of copper, nickel, aluminum and beryllium in the following ranges, 2.0% to 7.0% nickel; 0.5 to 2.0% aluminum; 0.25% to 1.25% beryllium, and the balance copper, wherein the nickel content exceeds the sum total of the aluminum and beryllium content. 55

9. A manufacture of hard beryllium copper alloys which comprises subjecting an alloy containing 2 to 7% of nickel; 0.5 to 2% of aluminum; 0.25 to 1.25% of beryllium, the balance of the 60 alloy consisting of copper, and the nickel content being about 3 1/2 times the aluminum content, to heat treatment involving heating the alloy to a temperature of the order of 800° C. followed by rapid cooling and reheating to a temperature of about 250°-550° C. 65

10. A manufacture as set forth in claim 9, in which the alloy, after rapid cooling from the temperature of the order of 800° C. is subjected to cold working prior to reheating. 70